

(No Model.)

A. HAMPRECHT.

MANUFACTURE OF DECORATED GLASSWARE.

No. 337,325.

Patented Mar. 2, 1886.

Fig. 1



Fig. 2.



Witnesses:  
J. A. Burns,  
H. S. Converse

August Hamprecht  
by his atty's  
Bakerwell & Koenig

## UNITED STATES PATENT OFFICE.

AUGUST HAMPRECHT, OF WELLSBURG, WEST VIRGINIA.

## MANUFACTURE OF DECORATED GLASSWARE.

SPECIFICATION forming part of Letters Patent No. 337,325, dated March 2, 1886.

Application filed December 16, 1885. Serial No. 185,797. (No specimens.)

*To all whom it may concern:*

Be it known that I, AUGUST HAMPRECHT, of Wellsburg, in the county of Brooke and State of West Virginia, have invented a new and useful Improvement in the Manufacture of Decorated Glassware; and I do hereby declare the following to be a full, clear, and exact description thereof.

My invention in the decoration of glassware consists of a new combination of the process of applying and burning on colors with that of grinding, whereby any desired party-colored design, pattern, or figure may be produced upon an article of glassware with novel and striking effect. The outlines, together with such other lines and parts as are desired to give strength and character to the design or pattern, are made by cutting or grinding, and are of a translucent character, the article being made of clear glass. The body of the design or parts of the same is colored by painting or otherwise; and the colors are fired or baked in. The result is a beautiful and unique decoration. It is applicable to any kind of glassware.

To enable others skilled in the art to make use of my invention, I will now describe it by reference to the accompanying drawings, in which—

3c. Figure 1 is a pitcher illustrating the process. Fig. 2 is a view of a piece of glass, showing another pattern.

The design shown in Fig. 1 is that of a vine having leaves and a flower. The vine *a*, stipules *b*, edges of the leaves *c* and flower *d*, and the veins *e* of the leaves are all formed by grinding, and are translucent, having a frosted appearance. The colored central portions, *f*, are produced by painting or varnishing, or by dusting on fusible coloring-matter, after which the article is placed in a suitable oven and the color fixed by burning or baking.

Any desired number and arrangement of the colors may be adopted, that depending entirely on the character of the design and the taste of the decorator.

In Fig. 2 I show a piece of glass upon which is a morning-glory. Here the stem *g*, calix *h*, and veins *i* are delineated by grinding, while the corolla or petals *k* are delineated by colors

or tints, whereby the delicate hues can be properly represented.

The process is conducted in the following manner: Any desired article of glassware is taken and color applied in spots at the proper points—for instance, for the leaves *c* and flower *d*. This color may be of one or more tints, as may be desired. The proper surfaces being thus covered, the article is placed in a suitable furnace, and the color or colors fixed by baking or burning. It is then taken to the cutting-shop and the edges of the colored spots ground to form the frosted edges of the leaves *c* and flower *d*. The figures thus made have colored centers and ground outlines. The connecting-lines in Fig. 1, the vine *a*, stipules *b*, and veins *e* necessary to complete the general design are ground in. It is apparent that designs of a great variety can be produced in this way. The wide or body portions are made by first applying a spot of color, and then the outline of the figure is cut, as stated, removing any part of the colored surface that may extend to the lines of cut. Party-colored designs can be produced on glassware in this way with beautiful and striking effects. The application of all kinds of flowers, leaves, plants, fruits, insects, geometrical and other figures, faces, and emblems to glassware by this process is contemplated.

It will be noticed that the ground edges of the leaves *c*, and the center and edges of the flower *d*, as well as the calix *h*, are composed of a series of surfaces or plane figures, *x*, having an imbricated appearance and a diagonal grain. This is accomplished by presenting the article to the wheel at an angle to the axis of the figure and overlapping the mark of the previous cut. This method is useful in representing scaly and other imbricated patterns. It gives a very handsome effect.

The coloring need not cover the entire surface of the clear glass in the bounds of the design, but may be put on portions only of the same.

What I claim as my invention, and desire to secure by Letters Patent, is—

1. The process of decorating glassware, which consists in applying and baking coloring-matter to the surface at the desired point, and too

then grinding the outlines of the desired figure or pattern around said colored surface, whereby a colored figure with frosted edges or outline is formed on the surface of the article, substantially as and for the purposes described.

2. The process of decorating glassware, which consists in applying and baking coloring-matter to the surface at the desired point, and then producing the cutline in frosted imbricated surfaces by grinding around said colored

surface, whereby a colored figure with a frosted imbricated outline is formed on the surface of the article, substantially as and for the purposes described.

In testimony whereof I have hereunto set my hand this 8th day of December, A. D. 1885.

AUGUST HAMPRECHT.

Witnesses:

SARAH E. McCORD,

G. W. McCORD.